

June 21, 1938.

R. T. K. CORNWELL

2,121,021

METHOD OF PRINTING AND ARTICLE RESULTING THEREFROM

Filed Aug. 23, 1935

FIG. 1.



FIG. 2.



FIG. 3.



FIG. 4.



INVENTOR

RALPH T. K. CORNWELL

BY

Watson, Bristol, Johnson & Leavenworth  
ATTORNEYS

## UNITED STATES PATENT OFFICE

2,121,021

## METHOD OF PRINTING AND ARTICLE RESULTING THEREFROM

Ralph T. K. Cornwell, Fredericksburg, Va., assignor to Sylvania Industrial Corporation, Fredericksburg, Va., a corporation of Virginia

Application August 23, 1935, Serial No. 37,526

8 Claims.

(Cl. 8—5)

The invention relates in general to the formation of indicia and in particular to a process of printing upon a pellicle of a hydrophilic colloid while in the gel condition, and includes correlated improvements designed to enhance the decorative character of the printed colloid.

Heretofore, indicia produced on articles formed of a hydrophilic colloid in the gel state by direct printing with an ink comprising an organic dyestuff have not been satisfactory. With the prior methods of direct printing, the dyestuff was found to be deposited chiefly on the surface, the deposit was not sufficiently dense and the edges of the indicia were diffuse. It has also been suggested to produce indicia on films of hydrophilic colloids while in a dry condition by direct printing with inks containing opaque pigments, such as titanium oxide. In this process, the deposit is formed only on the surface of the material, so that the indicia show very little adhesion to the base, and frequently bleed and flake off when the article is immersed in water.

It is a general object of the invention to provide articles formed of non-fibrous material capable of forming a hydrogel with an indicium which is characterized by being relatively permanent, strongly adherent when immersed in water and difficult to alter or remove, and a process for the production thereof.

A more specific object of the invention is to provide shrinkable container closures, formed of a hydrophilic colloid, with indicia comprising a dense deposit of color having a substantial depth of penetration and sharpness of outline, and a process for the production of such closures.

Other objects of the invention will in part be obvious and will in part appear hereinafter.

The invention accordingly comprises the several steps and the relation of one or more of such steps with respect to each of the others, and the article possessing the features and properties which are exemplified in the following detailed disclosure, and the scope of the invention will be indicated in the claims.

According to the invention, an indicium of satisfactory density, depth and sharpness of outline may be produced on a non-fibrous material capable of forming a hydrogel and especially a hydrophilic colloid in the gel state by impregnating the colloid with a water-miscible swelling agent therefor and which is also a solvent for the dyestuff employed in the ink, and then printing the impregnated material with an ink or composition containing a substantive or direct dye-

stuff preferably carried in a water-miscible vehicle.

The expressions "gel state" and "gel condition" are employed herein to designate the condition of a pellicle of a hydrophilic colloid which has been impregnated with a water miscible swelling agent therefor and which is also a solvent for substantive dyestuffs.

For a more complete understanding of the nature and objects of the invention, reference should be had to the accompanying drawing, in which:

Fig. 1 is a diagrammatic representation of an apparatus for carrying out certain steps of the process;

Fig. 2 is an illustration of a seamless tube formed of a hydrophilic colloid which has been printed in accordance with the invention;

Fig. 3 is a view of a printed shrinkable closure band; and

Fig. 4 is a view of a printed shrinkable closure cap.

The process of the invention may be applied for printing various hydrophilic colloids in the gel state such, for example, as cellulose hydrate; those cellulose ethers which swell in water and dissolve in alkalies; gelatine, casein and the like. The cellulose hydrate may be derived from viscose solutions or solutions of cellulose in cuprammonia or in zinc chloride. The hydrophilic colloid may be in the form of sheets, films, hollow bodies such, for example, as capsules, or seamless, flexible tubing which is adapted to be used as sausage casings or which may be severed into short lengths to form shrinkable closure bands. The process is also applicable for printing non-fibrous materials which are capable of imbibing water and forming a hydrogel.

A suitable dyestuff solvent is one which is miscible with water, preferably hygroscopic, and capable of penetrating the hydrophilic colloid, such, for example, as polyhydric alcohols such as glycerine, ethylene glycol, diethylene glycol, and ethers of the glycols such as methyl, ethyl, butyl, etc., and organic nitrogen compounds derivable from ammonia, such, for example, as the amines, amides, tetraammonium compounds, especially the alkyl and hydroxyl derivatives of these compounds such as the ethanolamines. Thus, the article to be printed may be first conditioned by immersing it in a bath containing 50% of water and 50% of monoethyl ether of ethylene glycol. The dyestuff solvent which is incorporated in the gel may be the same as or different from that used in the ink. Further, since the ink vehicle

is water-miscible, the hydrogel may be impregnated with the entire ink vehicle, if desired, in lieu of impregnating it only with the dyestuff solvent.

5 Water adhering to the surface of the article after the solvent impregnation is removed before printing, preferably by drying the surface as by passing a blast of warm air thereover, but care should be taken that the gel is not dried throughout. Preferably the gel is printed while it is at a temperature higher than atmospheric to increase the rate of penetration of the dyestuff.

10 The surface-dry and conditioned gel is printed with an ink containing a substantive dyestuff, such as is used for the direct dyeing of cotton and other forms of cellulose, dissolved in a water-miscible solvent. Suitable dyestuffs are those known as benzo form, plutoform black, formyl colors, diamine-aldehyde colors, of which the following may be given as examples: benzo fast red L and GL, benzo fast yellow, benzo pure blue, Columbia blue, benzo fast blacks, diamine deep black, oxydiamine black.

15 The dyestuff is selected so as to have a high solubility in the water-miscible solvent and a relatively low solubility, or to be insoluble, in water. Preferably there is used a dyestuff of which the fastness to light and water can be improved by a suitable after-treatment such, for example, as a treatment with an aqueous formaldehyde solution. In some cases the stability of the dyestuff to light and water may be increased further by treatment with copper sulphate or potassium dichromate. It is preferable to wash the dyestuff thoroughly in order to remove inorganic salts which are commonly present therein. If such salts are permitted to remain in the dyestuff, they tend to crystallize within the material and detract from the strength and transparency of the hydrophilic colloid.

20 The dyestuff is carried in a water-miscible vehicle containing a water-miscible solvent for the dyestuff, water, and preferably also an organic hygroscopic agent which may be also a solvent of the dyestuff. The water in the ink vehicle promotes the penetration of the dyestuff into the hydrogel structure. For the hygroscopic agent there may be employed a non-crystalline organic substance, for example a polyhydric alcohol, such as glycol, glycerine, or diethylene glycol; triethanolamine; and other known hygroscopic agents. If desired, the ink may be thickened by the addition of a thickening agent such as a gum, dextrose, starch, and the like.

25 By way of illustration, the following examples of a suitable ink composition are presented:

|                                  | Ink vehicles |         |         |         |         |
|----------------------------------|--------------|---------|---------|---------|---------|
|                                  | Percent      | Percent | Percent | Percent | Percent |
| Triethanolamine                  | 60           |         |         |         |         |
| Butyl ether of diethylene glycol |              | 70      | 50      | 50      |         |
| Methyl ether of glycol           |              | 60      |         |         | 10      |
| Diethylene glycol                |              | 20      | 20      | 20      |         |
| Water                            | 40           | 20      | 30      | 30      | 20      |

30 One of the above vehicles may be saturated with a direct or substantive dyestuff, such as benzoform BBL, benzoform orange and benzoform green FFL.

35 The process of the invention may be illustrated by reference to Fig. 1, in which an endless tube 1 of cellulose hydrate is passed from the supply roll 2 through a vat 3 which may contain a mixture of about 50 parts of monoethyl ether of

ethylene glycol and about 50 parts of water, the solution being maintained at a temperature of about 40° C. The surface liquid is removed from the tube as it passes between squeegee rollers 4.

40 The tube conditioned with the solvent then passes through the printing unit designated generally as 5, which comprises a heated roller 6, a pair of printing rollers 7 and 8 between which the tube passes, the roller 8 being provided with a raised design to which ink is applied from the inking rollers 9 and 10, the latter of which dips into the vessel 11 containing the ink.

45 After the printing operation, the printed material may be and preferably is aged for a time sufficient to produce the desired penetration of the dyestuff into the hydrogel. The penetration may be accelerated, for example by heating the printed material for about one minute or longer according to the penetration desired. Thus, the printed tube may be passed into and festooned in a chamber 12 heated to from 60° to 90° C. the traverse being completed in one minute. In lieu of heating, the material may be allowed to stand in air for a longer period of time. During the ageing, the dyestuff solvent should not be completely removed. Further, the penetration of the dyestuff is promoted by the presence of the solvent in the hydrogel.

50 Immediately after the ageing operation, the printed tube may be and preferably is immersed in a salt solution which renders the dyestuff insoluble and thus prevents smearing and bleeding of the indicia. For example, the tube may be passed through a vat 13 containing a 5%-10% aqueous solution of calcium chloride. After the salt treatment, the printed tube may be passed into a vat 14 containing water which washes off any excess ink and extracts the residual dyestuff solvent.

55 The printed material may now be placed in a vat 15 containing a 3% aqueous solution of formaldehyde maintained at a temperature of from 60° to 90° C. for about 30 minutes. The tube is then given a final washing in a vat (not shown) containing water and a small amount of an alkali to neutralize any acid remaining in the material. The printed and washed tube, which is still in a gel state, may be employed as sausage casing, and in this event it is subjected to the usual softening and drying treatments.

60 Alternatively, the printed tube 1 may be severed along the lines 16-16', as shown in Fig. 2, to form a shrinkable closure band 17, such as that illustrated in Fig. 3. When destined for use as bands, it is preferable to cut the tube as soon as possible after the printing operation, for example, at the point C shown in Fig. 1. The subsequent treatments of ageing, salting, washing and fixing may then be carried out as separate batch operations.

65 It is to be understood that the process is not restricted to the printing of seamless tubing, but is equally applicable for the printing of sheets, films, and hollow bodies such as capsules, in particular shrinkable closure caps 18, as shown in Fig. 4.

70 Since certain changes in carrying out the above process, and certain modifications in the article which embodies the invention may be made without departing from its scope, it is intended that all matter contained in the above description shall be interpreted as illustrative and not in a limiting sense.

75 It is also to be understood that the following claims are intended to cover all of the generic and

specific features of the invention herein described, and all statements of the scope of the invention which, as a matter of language, might be said to fall therebetween.

5. I claim:—

1. A process for producing an indicium on a pellicle of a hydrophilic colloid, comprising impregnating such a colloid with an organic water-miscible dyestuff solvent which is a swelling agent

10 for said colloid and printing the thus impregnated colloid in gel state with an ink containing a substantive dyestuff soluble in said solvent.

2. A process for producing an indicium on a pellicle of a hydrophilic colloid, comprising impregnating such a colloid with an organic water-miscible dyestuff solvent which is a swelling agent for said colloid and printing the thus impregnated colloid in gel state with an ink containing a substantive dyestuff soluble in said solvent and a water-miscible solvent therefor.

20 3. A process for producing an indicium on a pellicle of a hydrophilic colloid, comprising impregnating such a colloid with an organic water-miscible dyestuff vehicle which is a swelling agent for said colloid, printing the thus impregnated colloid in gel state with an ink containing a substantive dyestuff soluble in said vehicle and a water-miscible vehicle therefor, and thereafter fixing said dyestuff in the colloid.

25 4. A process for producing an indicium on a pellicle of a hydrophilic colloid, comprising impregnating such a colloid with an organic water-miscible dyestuff solvent which is a swelling agent for said colloid, printing the thus impregnated colloid in gel state with an ink containing a substantive dyestuff soluble in said solvent and a water-miscible solvent therefor, ageing the printed material whereby the dyestuff is diffused, and thereafter fixing the dyestuff.

5. A process for producing an indicium on a pellicle of a hydrophilic colloid, comprising impregnating such a colloid with an organic water-miscible dyestuff solvent which is a swelling agent for said colloid and printing the thus impregnated colloid in gel state in the presence of heat with an ink containing a substantive dyestuff soluble in said solvent and a water-miscible solvent therefor.

10 6. A process for producing an indicium on a pellicle of a hydrophilic colloid, comprising impregnating such a colloid with an organic water-miscible dyestuff solvent which is a swelling agent for said colloid, removing surface liquid from said impregnated colloid, heating and printing 15 said impregnated colloid in gel state with an ink containing a substantive dyestuff soluble in said solvent and a water-miscible solvent therefor, ageing the printed material and insolubilizing the dye impregnated in said material.

20 7. A process for producing an indicium on a pellicle of a non-fibrous material capable of forming a hydrogel, comprising impregnating said material with an organic water-miscible dyestuff solvent which is a swelling agent for said material, printing the thus impregnated material in gel state with an ink containing a substantive dyestuff soluble in said solvent, ageing said impregnated material, thereafter washing and fixing 25 said dyestuff in the material.

30 8. A process for producing an indicium on a pellicular article formed of cellulose hydrate, comprising impregnating such an article with an organic water-miscible dyestuff solvent which is a swelling agent for cellulose hydrate and then 35 printing said article in gel state with an ink containing a substantive dyestuff soluble in said solvent and a water-miscible solvent therefor.

RALPH T. K. CORNWELL.